

# UNITED STATES PATENT OFFICE.

GEORGE M. COLVOCORESSES, OF NEW YORK, N. Y.

## PROCESS OF MANUFACTURING IRON ALLOYS.

1,106,785.

Specification of Letters Patent. Patented Aug. 11, 1914.

No Drawing.

Application filed June 12, 1913. Serial No. 773,842.

To all whom it may concern:

Be it known that I, GEORGE M. COLVOCORESSES, a citizen of the United States of America, and residing at New York, in the county of New York and State of New York, have invented new and useful Improvements in Processes of Manufacturing Iron Alloys, of which the following is a specification.

10 The main object of the present invention is to provide for the commercial manufacture of an iron alloy at a low cost. This I do from ores whose iron content has been heretofore considered unavailable.

15 By my process I make an iron-nickel-copper alloy and a nickel-copper alloy steel direct from the ores containing iron, copper and nickel as sulfids. The resultant alloy is homogeneous in composition, is of a whitish color, is less corrosive than ordinary steel, has great mechanical strength, and can be rolled into sheets, plates, rods, rails, armor plates and drawn into wire or cast for other purposes; and can be produced more cheaply by this process than any other method known.

20 As examples of the ores which I propose to treat according to my invention I may mention the following compositions.

|                                           | No. 1,<br>basic. | No. 2,<br>medium.         | No. 3,<br>silicious. |
|-------------------------------------------|------------------|---------------------------|----------------------|
| Iron, Fe.                                 | 50.              | 40%                       | 40.                  |
| Sulfur, S.                                | 29.              | 25%                       | 20.                  |
| Nickel, Ni.                               | 1.5              | 2%                        | 2.5                  |
| Copper, Cu.                               | .4               | .8%                       | 1.                   |
| Silica, SiO <sub>2</sub> .                | 10.              | 20.                       | 32.                  |
| Magnesia, MgO.                            |                  |                           |                      |
| Lime, CaO.                                |                  |                           |                      |
| Alumina, Al <sub>2</sub> O <sub>3</sub> . |                  | Small varying quantities. |                      |

30 To make the alloy directly from the ore containing iron, nickel and copper as sulfids, the following process is employed:

40 (1) The ore is first crushed by rock breaker and pulverizing mill, such as a ball mill, to the desired degree of fineness which I find to be below 20-mesh.

(2) The crushed ore is next roasted with 45 suitable fuel in a standard roasting furnace, such as the McDougall, Herreshoff, or Wedge, until it is nearly or quite free from sulfur, and the iron, nickel and copper, which occurred as sulfids in the ore are converted wholly or in greater part into oxids.

50 In this roasting I employ sufficient fuel to remove all but the last 1% or so of sulfur.

(3) The roasted ore is then removed from the roasting furnace preferably while still hot and is suitably smelted with a suitable flux into a copper nickel ferro pig slaging

off the various non-metallic elements as silicates.

(4) The resultant copper-nickel ferro pig is then charged into an electric refining furnace or an open hearth furnace or Bessemer converter, and the remaining sulfur, silicon, excess carbon and other impurities are removed, the resultant material being a nickel-copper steel containing such percentage of carbon, as may be found most suitable and a combined content of copper and nickel from 1.5% to 12% according to the original composition of the ores treated which may be mixed as desired. Additional iron may be put in the refining furnace whenever it is found desirable to do so.

The process therefore contemplates first crushing the nickel-copper-iron ores to a suitable fineness; second, roasting out most 75 of the sulfur and converting the sulfids to oxids; third, smelting to remove most of the non-metallic elements; and fourth, refining to eliminate the remaining undesirable elements. The iron, nickel and copper are 80 kept together throughout the process.

The third step may be accomplished by smelting with a limestone flux in an electric shaft furnace. This third step may also be divided into two sub-steps—(a) nodulizing 85 by a suitable process, the gangue being used as a binder and lime added if necessary; (b) the nodulized ore is then charged into a blast furnace together with coke, limestone and such other flux as may be advisable and 90 the ore is smelted to a copper nickel ferro pig. The proportions of metals by weights in the said alloy steel will be within the following range:—Nickel—1 to 8%; copper—.5 to 4%; iron—82 to 98%. There will also 95 be present a limited amount of carbon up to 2% as may be found expedient for special purposes and such amount of impurities as would ordinarily exist in commercial steel and in nickel and copper. Examples of 100 alloys produced from the ores previously mentioned might contain the following percentages:—

|     | No. 1. | No. 2. | No. 3. |     |
|-----|--------|--------|--------|-----|
| Fe. | 98.35  | 94.8   | 91.4   | 105 |
| Ni. | 2.8    | 4.     | 6.     |     |
| Cu. | .75    | 1.     | 2.2    |     |
| C.  | .1     | .2     | .4     |     |

As an example of approximate physical properties of my alloy steel, the following may be cited:—A test bar of alloy steel with 110 6% nickel and 2% copper has approximately the following properties:—Ultimate

stress—108,000 lbs. per sq. in.; yield point—92,000 lbs. per sq. in.; reduction of area—50%; elongation 20%. It is not my intention however to limit my patent to the portions quoted above. This copper-nickel-steel will have practically the same physical properties as nickel-steel containing the same percentage of nickel as of combined copper and nickel in my steel and will be especially desirable for steel rails, armor plate, bridge rods, etc. The described method of production is simple, direct, inexpensive and tends to conserve the resources of the country, since in so far as possible, all of the iron, copper and nickel contained in the original ores are retained in the finished product.

By using the naturally complex iron-nickel copper ore and retaining all three elements together throughout the entire treatment I insure the most homogeneous and hence most valuable alloy of the three metals which it is possible to produce.

I have used the term iron alloy in a broad sense to include steel containing various percentages of carbon. The preferred product is an iron, nickel, copper, carbon alloy or a nickel, copper alloy steel.

It will be obvious that for commercial reasons the different steps of my process may be carried out in different places. For instance, the ore may be crushed, roasted and smelted at one place and the resultant pig shipped to another place for refining.

35 What I claim is:—

1. The process of making an iron alloy which consists in first crushing a nickel-copper-iron sulfid ore to a suitable fineness; second roasting out most of the sulfur and 40 converting the sulfids to oxids; third smelting to remove most of the non-metallic elements and to reduce the metallic oxids; and fourth refining to eliminate the remaining undesirable elements and retaining substan-

tially all of the iron, nickel and copper in 45 combination throughout the process.

2. The process of making an iron alloy which includes roasting a nickel, copper, iron sulfid ore to eliminate sulfur and form iron, copper and nickel oxids and then smelting 50 the product with a suitable flux to eliminate the non-metallic elements as silicates and to reduce the oxids to a pig of iron, nickel and copper suitable for subsequent refining.

3. The process of making an iron alloy 55 which consists in first crushing a nickel-copper-iron sulfid ore to a suitable fineness; second roasting out most of the sulfur and converting the iron, nickel and copper sulfids to oxids; and third smelting with a suitable 60 flux to remove most of the non-metallic elements and to reduce the metallic oxids to a pig of iron, nickel and copper suitable for refining.

4. The process of making a steel alloy 65 which includes roasting a nickel, copper, iron sulfid ore to eliminate sulfur and form iron, copper and nickel oxids and then smelting the product with a suitable flux to eliminate the non-metallic elements as silicates 70 and to reduce the oxids to a pig of iron, nickel, copper and carbon and then subsequently refining the composite pig and forming a nickel, copper alloy steel.

5. The process of making an iron alloy 75 which includes roasting a nickel-copper-iron sulfid ore containing from .5 to 12% nickel, from .2 to 10% copper, and from 25 to 60% iron and converting the iron, nickel and copper sulfids to oxids; and smelting with a 80 suitable flux to remove most of the non-metallic elements and to reduce the metallic oxids to a composite pig of iron, nickel and copper suitable for refining.

GEORGE M. COLVOCORESSES.

Witnesses:

ROBT. S. ALLYN,  
E. BRADFORD.